

# United States Patent [19]

Barton et al.

[11] 3,907,736

[45] Sept. 23, 1975

[54] FINISHING AGENTS FOR TEXTILES

[75] Inventors: **Kenneth R. Barton; Raymond N. Vachon**, both of Kingsport, Tenn.

[73] Assignee: **Eastman Kodak Company**, Rochester, N.Y.

[22] Filed: **May 20, 1974**

[21] Appl. No.: **471,427**

[52] U.S. Cl. .... **260/29.4 R**; **260/850**; **260/849**; **428/254**; **428/272**

[51] Int. Cl.<sup>2</sup> .... **C08L 67/00**

[58] Field of Search ..... **260/850, 29.4**; **117/139.5 A**

## [56] References Cited

### UNITED STATES PATENTS

3,546,008 12/1970 Shields et al. .... **260/40 P**

|           |         |                    |            |
|-----------|---------|--------------------|------------|
| 3,631,136 | 12/1971 | Spiller .....      | 260/29.2 E |
| 3,652,583 | 3/1972  | Tajima et al. .... | 260/849    |
| 3,734,874 | 5/1973  | Kibler et al. .... | 260/29.2 E |

Primary Examiner—John C. Bleutge

Assistant Examiner—Arthur H. Koekert

Attorney, Agent, or Firm—Elliott Stern; Daniel B. Reece, III

[57]

## ABSTRACT

Aqueous blends of (1) a water-dissipatable linear copolyester; (2) an amino resin crosslinking agent; and (3) a poly(oxyethylene)-containing glycol are useful for modifying the hand of fabrics and for reducing the tendency of knitted and woven polyester containing fabrics to snag or pick on sharp or abrasive objects in wear.

10 Claims, No Drawings

## FINISHING AGENTS FOR TEXTILES

This invention relates to compositions useful as finishing agents for textile articles. More specifically, this invention relates to compositions useful as finishing agents for textile articles containing polyester fibers. The compositions of this invention are useful for modifying the "hand" or "handle" of polyester fabrics as well as reducing the tendency of knitted and woven fabrics constructed from texturized polyester yarns to 10 snag or pick on sharp or abrasive objects during wear.

Knitted and woven fabrics constructed from texturized polyester yarns or yarns containing polyester fibers have the unfortunate tendency to snag or pick during normal wear. Snags detract from the appearance of 15 garments and shorten acceptable wear-life. The hand or handle of polyester-containing fabrics, particularly those containing only texturized polyester yarns, is also difficult to modify permanently with conventional finishing agents in that many have a tendency to lose their 20 finish during dry cleaning and washing procedures.

It is an object of this invention to provide compositions useful as finishing agents that impart a durable handle to textile articles containing polyester fibers and that reduce the tendency of fabrics constructed from 25 texturized polyester yarns to snag or pick on sharp or abrasive objects in wear. It is a further object of this invention to provide crosslinkable, aqueous blends when applied to fabrics which provide excellent adhesion to polyester and many other fibrous substrates, good wash 30 resistance, excellent dry cleaning resistance, and excellent handle. It is a further object of this invention to provide novel compositions which have applications in the areas of spray binding for staple fibers as a nonwoven fabric binder, a knit fabric hand builder, an antipick resin, a flocking adhesive and a fabric finish.

Water-dissipatable copolymers derived from at least one dicarboxylic acid component, at least one diol component, at least 20 mole percent of said diol being 40 a poly(ethylene)glycol, and a difunctional monomer containing a  $-\text{SO}_3\text{M}$  group wherein M is a monovalent alkali metal are disclosed in U.S. Pat. Nos. 3,734,874, 3,546,008 and 3,779,993. Furthermore, aqueous dispersions of coating compositions consisting of the 45 above type copolymers dispersed together with a melamine-formaldehyde resin have been sold under the trade name of WDX-743, WDX-744 and Eastman Binder DFB, products of Eastman Kodak Company. These aqueous coating compositions, however, provide coatings which produce a very stiff, unpleasant hand or 50 feeling to polyester fabrics. The compositions of this invention improve over the prior art compositions in that they impart a durable handle to textile articles and have advantageous picking and snagging properties.

In one aspect of this invention there is provided textile finishing agents which are prepared from aqueous blends of (1) a water dissipatable linear copolyester of the type disclosed in U.S. Pat. No. 3,734,874 and U.S. Pat. No. 3,546,008, (2) an amino crosslinking resin, and (3) a polyoxyethylene containing glycol. An acid or latent acid catalyst is used to effect a thermally-induced crosslinking reaction which, when carried out on the surface of textile fibers, leaves a water-insoluble film having good adhesion to textile fibers. The compositions thus formed, which partially or wholly covers the fiber surfaces and in some instances forms inter-fiber bonds, imparts an illusion of added weight and

bulk to the fabric and reduces the tendency of the fabric to snag or pick. The handle of the finished fabric may be controlled by judicious selection of the ratio of the three components in finishing agent formulation as hereinafter described.

The compositions of this invention can be more specifically defined as an aqueous blend of the following components:

1. from about 50 to about 85 (preferably about 70 to about 80) parts by weight of a linear, water-dissipatable polyester derived from components (A), (B) and (C) as follows:
  - A. at least one dicarboxylic acid,
  - B. at least one diol, at least 20 mole percent of said diol component being a poly(ethylene)glycol having the formula  $\text{H}-\text{OCH}_2\text{CH}_2)_n\text{OH}$  wherein n is an integer of from 2 to about 14, and
  - C. at least one difunctional dicarboxylic acid sulfomonomer containing a  $-\text{SO}_3\text{M}$  group attached to an aromatic nucleus, wherein M is  $\text{Na}^+$ ,  $\text{Li}^+$ ,  $\text{K}^+$ , or a combination thereof, said sulfomonomer component constituting at least about 8 mole percent to about 45 mole percent of the sum of the moles of said components (A) and (C);
2. from about 15 to about 50 (preferably about 20 to about 30) parts by weight of at least one water-dissipatable amino resin having at least two reactive groups, said resin being selected from the group consisting of melamine-formaldehyde condensates, methylated melamine-formaldehyde condensates, urea-formaldehyde condensates, methylated urea-formaldehyde condensates, guanamine-formaldehyde condensates and methylated guanamine-formaldehyde condensates; and
3. from about 10 to about 100 (preferably about 10 to about 60) parts by weight of a water-dissipatable nonionic linear poly(oxyethylene) containing glycol having the formula (I)  $\text{HO}-(\text{CH}_2\text{CH}_2\text{O})_m\text{H}$  wherein m is an integer from about 4 to about 150, or



wherein x, y, and z are integers, the sum of which results in a glycol having a molecular weight from about 1,000 to about 14,000, and the ratio of x + z to y is such that the hydrophile/lipophile balance is from about 4.5 to about 30.5.

In one preferred embodiment of this invention the above aqueous blends contain about 0.5 to about 50 percent by weight of combined solids supplied by components 1, 2) and 3).

The dicarboxylic acid component (A) from which the linear water-dissipatable polyester component of this invention is prepared can be any aliphatic, cycloaliphatic, or aromatic acid. Examples of such dicarboxylic acids include oxalic; malonic; dimethylmalonic; succinic; glutaric; adipic; trimethyladipic; pimelic; 2,2-dimethylgutaric; azelaic; sebacic; fumaric; maleic; itaconic; 1,3-cyclopantanedicarboxylic; 1,2-cyclohexanedicarboxylic; 1,3-cyclohexanedicarboxylic; 1,4-cyclohexanedicarboxylic; phthalic; terephthalic; isophthalic; 2,5-norbornanedicarboxylic; 1,4-naphthalic; diphenic; 4,4'-oxydibenzoic; diglycolic; thiadipropi-

onic; 4,4'-sulfonyldibenzoic; and 2,5-naphthalenedicarboxylic acids. In a preferred embodiment of this invention isophthalic acid is the dicarboxylic acid utilized. If terephthalic acid is used as the dicarboxylic acid component of the polyester, especially good results are achieved when at least five mole percent of one of the other acids listed above is used.

It should be understood that the use of the corresponding acid anhydrides, esters, and acid chlorides of these acids is included in the term "dicarboxylic acid." The esters are preferred, examples of which include dimethyl 1,4-cyclohexanedicarboxylate; dimethyl 2,6-naphthalenedicarboxylate; dibutyl 4,4'-sulfonyldibenzoate; dimethyl isophthalate; dimethyl terephthalate; and diphenyl terephthalate. Copolymers may be prepared from two or more of the above dicarboxylic acids or derivatives thereof.

At least about 20 mole percent of the diol component (B) used in preparing the water-dissipatable polyester component of the invention is a poly(ethylene)glycol having the formula  $H-OCH_2CH_2-OH$  wherein  $n$  is an integer of from two to about ten. Examples of suitable poly(ethylene)-glycols include diethylene, triethylene, tetraethylene, pentaethylene, hexaethylene, heptaethylene, octaethylene, nonaethylene, and decaethylene glycols, and mixtures thereof. Preferably the poly(ethylene)glycol employed in the polyester of the present invention is diethylene glycol, triethylene glycol, or mixtures thereof. The remaining portion of the diol component is at least one aliphatic, cycloaliphatic, or aromatic diol. Examples of these diols include ethylene glycol; propylene glycol; 1,3-propanediol; 2,4-dimethyl-2-ethylhexane-1,3-diol; 2,2-dimethyl-1,3-propanediol; 2-ethyl-2-isobutyl-1,3-propanediol; 1,3-butanediol; 1,4-butanediol; 1,5-pantanediol; 1,6-hexanediol; 2,2,4-trimethyl-1,6-hexanediol; 1,2-cyclohexanediethanol; 2,2,4,4-tetramethyl-1,3-cyclobutanediol; and p-xylylenediol. Copolymers may be prepared from two or more of the above diols.

The third component (C) used to prepare the water-dissipatable polyester is a difunctional monomer containing a  $-SO_3M$  group attached to an aromatic nucleus, wherein M is hydrogen or a metal ion. This difunctional monomer component may be either a dicarboxylic acid (or derivative thereof) containing a  $-SO_3M$  group or a diol containing a  $-SO_3M$  group. The metal ion of a sulfonate salt group may be  $Na^+$ ,  $Li^+$ , or  $K^+$ .

The  $-SO_3M$  group is attached to an aromatic nucleus, examples of which include benzene, naphthalene, anthracene, diphenyl, oxydiphenyl, sulfonyldiphenyl, and methylenediphenyl.

Especially good results are obtained when the difunctional monomer is the sodium salt of a sulfoisophthalic, sulfoterephthalic, sulfophthalic, or 4-sulfonaphthalene-2,7-dicarboxylic acid (or derivatives of such acids). A highly preferred monomer is 5-sodiosulfoisophthalic acid or derivative thereof such as 5-sodiosulfodimethyl isophthalate.

Other effective difunctional monomers containing a  $-SO_3M$  group attached to an aromatic nucleus include metal salts of aromatic sulfonic acids (or esters thereof). These monomers have the general formula



wherein X is a trivalent aromatic hydrocarbon radical, Y is a divalent aromatic hydrocarbon radical, R is hydrogen or an alkyl group of one to four carbon atoms, M is  $Na^+$ ,  $Li^+$ , or  $K^+$ , and  $a$  is 1, 2 or 3. These monomers are described, including methods for their preparation, in U.S. Pat. No. 3,528,947, patented on Sept. 15, 1970. Examples of preferred monomers are 4-sodiosulfophenyl-3,5-dicarbomethoxybenzene-sulfonate, 4-lithiosulfophenyl-3,5-dicarbomethoxybenzenesulfonate; and 6-sodiosulfo-2-naphthyl-3,5-dicarbomethoxybenzenesulfonate.

Other effective difunctional monomers containing a  $-SO_3M$  group attached to an aromatic nucleus include metal salts of sulfodiphenyl ether dicarboxylic acids (or esters thereof). These monomers have the general formula



wherein R is hydrogen, an alkyl group of one to eight carbon atoms, or phenyl, M is  $Na^+$ ,  $Li^+$ , or  $K^+$ , and  $a$  is 1, 2, or 3. Examples of preferred monomers here are dimethyl 5-[4-(sodiosulfo)phenoxy]isophthalate, dimethyl 5-[4-(sodiosulfo)phenoxy]terephthalate, and 5-[4-(sodiosulfo)phenoxy]isophthalic acid.

The water-dissipatable polyester should contain at least about eight mole percent of the monomer based on total acid content, with about 10 mole percent giving particularly advantageous results. Greater dissipability is achieved when the difunctional monomer constitutes from about 10 mole percent to about 45 mole percent of the total content of acid of the polyester.

To obtain the polyester component of this invention, the difunctional monomer containing the  $-SO_3M$  group may be added directly to the esterification reaction mixture from which the polyester will be made. Thus, these monomers can be used as a component in the original polyester reaction mixture. Other various processes which may be employed in preparing these polyesters are well known in the art and are illustrated in such patents as U.S. Pat. Nos. 2,465,319; 3,018,272; 2,901,466; and 3,075,952. These patents illustrate ester interchange and polymerization processes.

Whenever the term "inherent viscosity" (I.V.) is used in this description, it will be understood to refer to viscosity determinations made at 25°C. using 0.5 gram of polymer per 100 ml. of a solvent composed of 60% phenol and 40% tetrachloroethane as parts by weight. In addition, whenever the terms "dissipatable," "dissipated" or "dissipate," are used in this description, it will be understood to refer to the action of water or aqueous solutions on the components of the blends of this invention. The terms are specifically intended to cover those situations wherein the solution dissolves and/or disperses these blends. Furthermore, whenever the word "water" is used in this description, it includes not only aqueous solutions but also hot aqueous solutions.

In an especially preferred embodiment of this invention the water-dissipatable polyester component is derived from 90 mole percent isophthalic acid, 10 mole percent of 5-sodiosulfoisophthalic acid, and 100 mole percent of diethylene glycol and having an inherent viscosity (I.V.) of at least 0.30 as measured at 25° using 0.50 gram of polymer per 100 ml. of a solvent composed of 60 percent phenol and 40 percent tetrachloroethane. The copolyester useful in this invention may be terminated with either hydroxy or carboxy end-groups. In addition, the end-group functionality of the copolyester, and therefore its crosslinkability, may be increased by reaction of the high molecular weight linear polyester with tri- or tetrafunctional hydroxy or carboxy compounds such as trimethylolpropane, pentaerythritol, or trimellitic anhydride in a manner known in the art.

Examples of the water-dispersible amino resins useful in this invention include the melamine-formaldehyde condensates, the methylated (wholly or partially) melamine-formaldehyde condensates, the urea-formaldehyde condensates, methylated (wholly or partially) urea-formaldehyde condensates, the methylated (wholly or partially) guanamine-formaldehyde condensates, and the like. These amino resins are known in the art and can be prepared by known means or obtained commercially. The properties of these resins, as well as some of their uses in textiles applications, are set forth in Mark, Wooding, and Atlas, *Chemical Aftertreatment of Textiles*, John Wiley & Sons, Inc. (1971), pages 267-355. Preferred amino resins useful in this invention are hexamethoxymethyl melamine (Cymel 300, a registered trademark of American Cyanamid Company), partially methylated melamine formaldehyde adduct sold also under various trade names (for example, Aerotex M-3, a registered trademark of American Cyanamid Company), and various urea-formaldehyde condensates such as Aerotex Resin 802, a registered trademark of American Cyanamid Company.

Examples of poly(oxyethylene) containing glycols useful in this invention are those which have an average molecular weight of from 200 to about 7,000, the only requirement being that the poly(oxyethylene)-glycols be dispersible in water. Especially preferred poly(oxyethylene)-glycols useful in this invention are those having an average molecular weight of from about 1000 to about 6000 (e.g., having the formula  $\text{HO}(\text{CH}_2\text{CH}_2\text{O})_n\text{H}$  wherein  $n$  is an integer of from about 20 to about 130), sold under the trade name Carbowax, a registered trademark of Union Carbide Corporation. Examples of the specific Carbowaxes useful in this invention are Carbowax 200, Carbowax 4000, and Carbowax 1000, Carbowax 4000 being especially preferred. Also useful as the poly(oxyethylene)glycol component of this invention are the water-dispersible ethylene oxide-propylene oxide block copolymer glycols which are also sold commercially under the trade name of Pluronics, a registered trademark of Wyandotte Chemicals Corporation. These glycols are the condensates of ethylene oxide with hydrophobic bases formed by condensing propylene oxide with propylene glycol and have the general formula



where  $x$ ,  $y$ , and  $z$  are integers, the sum of which results in molecular weights ranging from about 1,000 to 14,000, preferably 3,000 to 10,000. The ratio of  $x+z/y$  is such that the HLB (hydrophile/lipophile balance) is from about 4.5 to about 30.5, preferably 6.6 to 24.5. [The HLB of a nonionic surfactant is defined as the approximate weight percent of ethylene oxide in the surfactant divided by 5. See W. C. Griffin, *J. Soc. Cosmetic Chemists*, 1, 311 (1949).]

10 Examples of useful Pluronics are Pluronic F38, L35 and P65.

The ratio of poly(oxyethylene) containing glycol to combined parts of copolyester and amino resin used in the dispersions of this invention determines the softness 15 of the cured film and therefore the softness of the finished textile article. If no poly(oxyethylene)glycol is used, the finished article tends to be rather stiff and boardy. Softness increases with increasing poly(oxyethylene)glycol content. Surprisingly, it has been found 20 that the articles coated with the compositions of this invention show better softness or handle properties than the prior art compounds. In a preferred embodiment of the invention 10 to 60 parts by weight of poly(oxyethylene)glycol per 100 parts of copolyester-amino resin is used to produce commercially attractive 25 "hands" of increasing softness.

The optimum ratio of copolyester to amino resin depends upon several factors, including amino resin functionality and reactivity, copolyester end-group concentration and reactivity, and molecular weight and concentration of poly(oxyethylene)glycol. The copolyester/amino resin ratios found useful in practice of the invention range from about 1:1 to 6:1, the preferred ratio being about 3:1 copolyester/amino resin.

30 The above components 1), 2) and 3) are, for convenience in commercial handling, dispersed in enough water to bring the total solids content to approximately 30 percent. This concentration can then be readily diluted to the desired level for application to textile substrates when ready for use. It is desirable but not essential to include 1 to 10 parts (4 to 5 parts preferred) of a poly(oxyethylated) alkyl phenol to the 30 percent solid dispersion. This type of nonionic surfactant improves the storage life and electrolyte stability of the formulation and serves as a wetting agent for the substrate. Poly(oxyethylated) alkyl phenols are sold under various trade names, such as Triton, a registered trademark of Rohm & Haas Company, and Igepal, a registered trademark of GAF Corporation.

40 To apply a finish of the type disclosed in this invention to a textile substrate, a pad bath containing the desired component is prepared either by direct addition of the individual components to water or by dilution of a high solids (30 percent, for example) dispersion. The solids content of the pad bath is adjusted so as to obtain about 0.5 to 5 percent (1 to 3 percent preferred) add-on of finish on the fabric when dried. In order to accelerate the curing or crosslinking reaction which insolubilizes the finish on the fabric, it is necessary to include an acid or a latent acid catalyst in the pad bath. Generally, from 0.5 to 3 percent (based on weight of solids in the pad bath) of catalyst is sufficient to effect a cure 45 under typical textile processing conditions. The optimum catalyst concentration depends upon the catalyst used, the nature of the amino resin, and the time and temperature of curing. Examples of such suitable catalysts which may be used to promote the reaction of the

50

55

60

65

amino resin with the hydroxy or carboxy groups available in the dispersion are well known in the art and include p-toluenesulfonic acid, citric acid, glycolic acid, oxalic acid, amine hydrochloride, zinc fluoborates, and magnesium chloride. Citric acid and p-toluenesulfonic acid are preferred. Further examples of these useful catalysts are described in Mark, Wooding, and Atlas, *Chemical Aftertreatment of Textiles*, John Wiley & Sons (1971), pages 332-334. The optimum catalyst concentration depends upon the catalyst used, the nature of the amino resin, and the time and temperature of curing. For a given formulation the optimum catalyst and catalyst concentration are best determined by experimentation. The formulation containing catalyst is applied to the textile substrate by padding (dipping and nipping), by over-spray or by kiss role. The article is then dried and thermally cured by passing it through, for example, an oven or a bank of infrared heaters. No additional treatments are necessary, but the article may be afterwashed if desired.

The following examples illustrate the invention.

#### EXAMPLE 1

##### PREPARATION OF 30% CONCENTRATE

To 313 parts of warm (160°F.) demineralized water is added 75 parts of the 90/10 copolyester of isophthalic acid/5-sodiosulfoisophthalic acid and diethylene glycol (inherent viscosity 0.42), 25 parts of hexamethoxymethyl melamine (Cymel 300), 30 parts of poly(oxyethylene)glycol, average molecular weight 4000 (Carbowax 4000), and 4.2 parts of Igepal CO 970 (GAF Corp.). The mixture is stirred until all materials have either dissolved or dispersed in the water medium.

#### EXAMPLE 2

##### APPLICATION OF FINISH TO FABRIC

A portion of the 30% concentrate from Example 1 is diluted 10-fold with demineralized water (3% final bath

solids). To 500 g. of the diluted formulation is added 0.45 g. of citric acid (3% catalyst based on weight of bath solids). A 100% textured polyester (150 denier) double-knit fabric (8 oz./sq. yd., Ponti de Roma style) is padded with the above formulation, dried at 220°F. for 10 minutes and cured at 340°F. for 90 seconds. The dry weight increase of the fabric is 2.1%. In comparison with the original, untreated fabric (heated in the same manner), the finished fabric feels considerably heavier and slightly stiffer. The handle of the treated fabric is not changed significantly by typical home laundering procedures. Resistance of the treated fabric to snagging as measured by the Mace Test (J. A. Finnigan, Textile Institute and Industry, pp. 164-167, June, 1972) is also increased. The Mace rating of the original fabric is 2.5, whereas the Mace rating of the treated fabric is 4.0. (5 = no snagging; 1 = very bad snagging).

#### EXAMPLE 3

Pad baths (approximately 3% total solids) containing the ingredients listed in Table 1 are prepared in the manner described in Examples 1 and 2 except 1% (on weight of solids) of p-toluenesulfonic acid catalyst is used instead of citric acid. Several 100% polyester fabrics are padded with the formulations shown so as to obtain about 2% dry add-on (based on initial fabric weight). The padded fabrics are dried at 220°F. and cured as shown in the table. Each fabric is evaluated for handle (subjective test) and snagging tendency as measured by the Mace Test. All of the treated fabrics appear subjectively to be heavier than the original, untreated fabrics and the original "handle" is not greatly changed by laundering.

Hydroxyl number of the polyester is defined as the number of milligrams of potassium hydroxide consumed per gram of sample in the titration of the acetic acid liberated by the reaction of acetic anhydride with the hydroxyl end groups of the polyester dissolved in pyridine.

Table 1

| Polyester, Parts | Amino Resin, Parts | Poly(oxyethylene)-Containing Glycol<br>Mol. Wt., Parts | Cure Time/Temp.<br>sec./°F. | Fabric Num-<br>ber | Fabric Handle   | Mace Rating |
|------------------|--------------------|--------------------------------------------------------|-----------------------------|--------------------|-----------------|-------------|
| 1                | 75                 | A 25 4000*                                             | 90/340                      | I                  | firm, dry       | 4.0         |
| 1                | 75                 | B 25 4000                                              | 90/340                      | I                  | soft, smooth    | 3.5         |
| 2                | 75                 | A 25 200**                                             | 240/300                     | II                 | soft, smooth    | 4.5         |
| 2                | 50                 | A 50 200                                               | 240/300                     | II                 | medium soft     | 4.0         |
| 3                | 85                 | B 15 6000***                                           | 90/340                      | III                | v. soft, smooth | 4.5         |
| 3                | 85                 | C 15 6000                                              | 60/355                      | III                | medium soft     | 4.0         |
| 1                | 75                 | A 25 2900****                                          | 90/340                      | I                  | medium soft     | 3.5         |
| 2                | 75                 | B 25 14000*****                                        | 90/340                      | I                  | crisp, smooth   | 3.5         |

Polyester 1 - 90/10 Copolyester of isophthalic/5-sodiosulfoisophthalic acids and diethylene glycol, inherent viscosity 0.42, hydroxyl number 14.

Polyester 2 - 45/45/10 Copolyester of isophthalic/adipic/5-sodiosulfoisophthalic acids and diethylene glycol, inherent viscosity 0.35, hydroxyl number 18.

Polyester 3 - Polyester 1 reacted with 3 weight percent trimethylol propane, inherent viscosity 0.25, hydroxyl number 41.

Aminoresin A - Hexamethoxymethyl melamine (Cymel 300).

Aminoresin B - Partially methylated melamine-formaldehyde condensate (Aerotex M-3 resin).

Aminoresin C - Urea-formaldehyde condensate (Aerotex 802 Resin).

Fabric 1 - Ponti de Roma double-knit, 8 oz./sq. yd., made from 150 denier textured continuous filament polyester yarn. Mace rating 2.5 after heat-setting (wales direction).

Fabric 2 - Patterned warp knit, 7.5 oz./sq. yd., made from 150 denier textured continuous filament polyester yarn. Mace rating 2.0 after heat-setting (warp direction).

Fabric 3 - Plain weave 90 x 60, 6 oz./sq. yd., made from 150 denier textured continuous filament polyester yarn (warp and filling). Mace rating (warp direction) 3.0 after heat-setting.

\*Carbowax 4000

\*\*Carbowax 200

\*\*\*Carbowax 6000

\*\*\*\*Pluronic L64, HLB 15.0

\*\*\*\*\*Pluronic F108, HLB 27.0

## EXAMPLE 4

A mixture of 48.5 grams (0.25 mole) of dimethyl isophthalate, 24.2 grams (0.125 mole) of dimethyl terephthalate, 15 grams (0.075 mole) of hexahydroisophthalic acid, 14.8 grams (0.05 mole) of dimethyl 5-sodiosulfoisophthalate, 68.9 grams (0.65 mole) of diethylene glycol, and 0.8 ml. of a 21 percent catalyst solution of titanium isopropoxide in isopropanol is stirred and heated at 200°C. and a vacuum of 0.3 mm. is applied. Heating and stirring is continued for one hour under these conditions. After cooling the polymer obtained has an I.V. of 0.53 and is tough and rubbery. To 313 parts of warm (160°F.) demineralized water is added 75 parts of the above copolyester, 25 parts of hexamethoxymethyl melamine (Cymel 300), 30 parts poly(oxethylene)glycol, average molecular weight about

2000 and 4.0 parts of Igepal CO 970. The mixture is stirred until all materials have either dissolved or dispersed in the water medium.

Example 2 is repeated with similarly advantageous results.

## EXAMPLE 5

The following Table II shows the properties of a number of water dissipatable polyesters made from difunctional monomers containing  $-\text{SO}_3\text{M}$  groups. All are made by the general procedure of Example 4. These polyesters are blended in with Carbowax 1000, a poly(oxethylene)-glycol having an average molecular weight of 1000 and Aerotex Resin M-3 in the manner disclosed in Example 1. When the aqueous blends thus formed are treated and applied to fabric as shown in Example 2, similarly advantageous results are obtained.

TABLE II

| Polymer | Dicarboxylic Acid     | Mole Percent | Sulfonate        | Mole Percent | Diol                              | Mole Percent | I.V. |
|---------|-----------------------|--------------|------------------|--------------|-----------------------------------|--------------|------|
| A       | Isophthalic           | 52.5         | SIP <sup>1</sup> | 17.5         | DEG <sup>2</sup>                  | 100          | 0.54 |
|         | Terephthalic          | 25           |                  |              |                                   |              |      |
|         | Hexahydroisophthalic  | 5            |                  |              |                                   |              |      |
| B       | Isophthalic           | 90           | SIP              | 10           | DEG                               | 100          | 0.53 |
|         | Hexahydroterephthalic | 90           |                  |              |                                   |              |      |
| C       | Isophthalic           | 90           | SIP              | 10           | (DEG<br>80)                       | 100          | 0.73 |
|         | Isophthalic           | 50           |                  |              |                                   |              |      |
|         | Terephthalic          | 25           |                  |              |                                   |              |      |
| D       | Isophthalic           | 15           | SIP              | 10           | (EG <sup>3</sup><br>20)           | 100          | 0.60 |
|         | Hexahydroisophthalic  | 50           |                  |              |                                   |              |      |
| E       | Terephthalic          | 25           | (4)              | 10           | DEG                               | 100          | 0.42 |
|         | Hexahydroisophthalic  | 15           |                  |              |                                   |              |      |
| F       | Isophthalic           | 90           | (5)              | 10           | DEG                               | 100          | 0.48 |
|         | Isophthalic           | 60           |                  |              |                                   |              |      |
| G       | Isophthalic           | 90           | (5)              | 10           | DEG                               | 100          | 0.55 |
|         | Hexahydroterephthalic | 30           |                  |              |                                   |              |      |
| H       | Isophthalic           | 90           | (6)              | 10           | DEG                               | 100          | 0.42 |
|         | Terephthalic          | 92           |                  |              |                                   |              |      |
| I       | Isophthalic           | 92           | SIP              | 8            | TEG <sup>7</sup>                  | 100          | 0.33 |
|         | Terephthalic          | 92           |                  |              |                                   |              |      |
| J       | Isophthalic           | 90           | SIP              | 10           | TEG                               | 100          | 0.59 |
|         | Isophthalic           | 90           |                  |              |                                   |              |      |
| K       | Isophthalic           | 90           | SIP              | 10           | (CHDM <sup>8</sup><br>(DEG<br>70) | 100          | 0.45 |
|         | Adipic                | 90           |                  |              |                                   |              |      |
| L       | Isophthalic           | 90           | SIP              | 10           | DEG                               | 100          | 0.69 |
|         | Isophthalic           | 90           |                  |              |                                   |              |      |
| M       | Isophthalic           | 90           | SIP              | 10           | (CHDM<br>(DEG<br>50)              | 100          | 0.48 |
|         | Isophthalic           | 90           |                  |              |                                   |              |      |
| N       | Isophthalic           | 90           | SIP              | 10           | (CHDM<br>(DEG<br>60)              | 100          | 0.51 |
|         | Isophthalic           | 80           |                  |              |                                   |              |      |
| O       | Isophthalic           | 80           | SIP              | 20           | (CHDM<br>(DEG<br>70)              | 100          | 0.32 |
|         | Isophthalic           | 80           |                  |              |                                   |              |      |
| P       | Isophthalic           | 80           | SIP              | 20           | (CHDM<br>(DEG<br>60)              | 100          | 0.38 |
|         | Isophthalic           | 80           |                  |              |                                   |              |      |

<sup>1</sup>SIP—5-sodiosulfoisophthalic acid.

<sup>2</sup>DEG—diethylene glycol.

<sup>3</sup>EG—ethylene glycol.

<sup>4</sup>4-sodiosulfonylphenyl-3,5-dicarboxybenzenesulfonate.



<sup>5</sup>5-[4-(sodiosulfo)phenoxy]isophthalic acid.



<sup>6</sup>2-(2'-sodiosulfonylphenyl)-2-ethylmalonic acid.



<sup>7</sup>TEG—triethylene glycol.

<sup>8</sup>CHDM—1,4-cyclohexanedimethanol.

Although the invention has been described in considerable detail with particular reference to certain preferred embodiments thereof, variations and modifications can be effected within the spirit and scope of the invention.

We claim:

1. An aqueous blend of components (1), (2) and (3) as follows:

1. from about 50 to about 85 parts by weight of a linear, water-dissipatable polyester derived from components A, B and C as follows:

A. at least one dicarboxylic acid,

B. at least one diol, at least 20 mole percent of said diol component being a poly(ethylene)glycol having the formula  $H-O(CH_2CH_2)_nOH$  wherein  $n$  is an integer of from 2 to about 14, and

C. at least one difunctional dicarboxylic acid sulfomonomer containing a  $-SO_3M$  group attached to an aromatic nucleus, wherein  $M$  is  $Na^+$ ,  $Li^+$ ,  $K^+$ , or a combination thereof, said sulfomonomer component constituting at least about 8 mole percent to about 45 mole percent of the sum of the moles of said components (A) and (C).

2. from about 15 to about 50 parts by weight of at least one water-dissipatable amino resin having at least two reactive groups, said resin being selected from the group consisting of melamine-formaldehyde condensates, methylated melamine-formaldehyde condensates, urea-formaldehyde condensates, methylated urea-formaldehyde condensates, guanamine-formaldehyde condensates and methylated quanamine-formaldehyde condensates; and

3. from about 10 to about 100 parts by weight of a water-dissipatable nonionic linear poly(oxyethylene)glycol having the formula (I)  $HO(CH_2C-H_2O)_mH$  wherein  $m$  is an integer from about 4 to about 150, or



wherein  $x$ ,  $y$ , and  $z$  are integers, the sum of which results in a glycol having a molecular weight from about 1000 to about 14,000 and the ratio of  $x+z$  to  $y$  is such that the hydrophile/lipophile balance is from about 4.5 to about 30.5.

2. The aqueous blends of claim 1 comprising

1. from about 70 to about 80 parts by weight of component (1);

2. from about 20 to about 30 parts by weight of components 2; and

3. from about 10 to 60 parts by weight of component (3).

3. The aqueous blend of claim 2 wherein component (1) is derived from

A. isophthalic acid,

B. 5-sodiosulfoisophthalic acid, and

C. diethylene glycol;

component (2) is selected from the group consisting of wholly methylated melamine-formaldehyde condensates, partially methylated melamine condensates, partially methylated urea-formaldehyde condensates and wholly methylated urea-formaldehyde condensates; and

component (3) is a polyethylene glycol having the formula  $HO(CH_2CH_2O)_mOH$  wherein  $m$  is an integer from 20 to about 130.

4. The aqueous blend of claim 1 containing 0.5 to about 50% by weight of the combined components (1), (2) and (3) based on the weights of components (1), (2) and (3) and water added together.

5. The aqueous blend of claim 2 containing 0.5 to about 50% by weight of the combined components (1), (2) and (3) based on the weights of components (1), (2) and (3) and water added together.

6. The aqueous blend of claim 3 containing 0.5 to about 50% by weight of the combined components (1), (2) and (3) based on the weights of components (1), (2) and (3) and water added together.

7. The aqueous blend of claim 4 containing 25 to about 35% by weight of the combined components (1), (2) and (3).

8. The aqueous blend of claim 5 containing 25 to about 35% by weight of the combined components (1), (2) and (3).

9. The aqueous blend of claim 6 containing 25 to about 35% by weight of the combined components (1), (2) and (3).

10. An aqueous blend of components (A), (B) and (C) as follows:

A. about 75 parts by weight of a linear water-dissipatable polyester derived from 90 mole percent isophthalic acid, 10 mole percent 5-sodiosulfoisophthalic acid and 100 mole percent diethylene glycol;

B. about 25 parts by weight of hexamethoxymethyl melamine; and

C. from about 20 to about 60 parts by weight of a poly(oxyethylene)glycol having an average molecular weight of about 4000.

\* \* \* \* \*